

April 26, 1938.

T. STEVENSON

2,115,047

TRACER AMMUNITION AND TO AN IGNITER MIXTURE FOR TRACER COMPOSITIONS

Filed Nov. 30, 1936



Inventors  
Thomas Stevenson  
Ernest R. Rechel  
By *W.N. Roach*  
Attorney

## UNITED STATES PATENT OFFICE

2,115,047

TRACER AMMUNITION AND TO AN IGNITER  
MIXTURE FOR TRACER COMPOSITIONSThomas Stevenson and Ernest R. Rechel,  
Philadelphia, Pa.

Application November 30, 1936, Serial No. 113,408

4 Claims. (Cl. 52—2)

(Granted under the act of March 3, 1883, as  
amended April 30, 1928; 370 O. G. 757)

The invention described herein may be manufactured and used by or for the Government for governmental purposes, without the payment to us of any royalty thereon.

5 This invention relates to tracer ammunition and igniter mixture for tracer compositions.

In tracer ammunition a combustible in a hollow bullet is ignited by the propellant charge and provides a visible trace, by means of smoke or

10 flame, from the moment the bullet leaves the gun until the combustible is completely consumed.

The visible indication of the initial trajectory of the bullet is a disadvantage in that, under 15 conditions of darkness, it discloses the position of the gun, and it confuses and misleads the gunner or fire director when aiming of the gun is accomplished by observation of the trace.

The objects of this invention are to provide 20 tracer ammunition in which the initial trajectory will not be visible and to secure the delayed action by employing a special igniter mixture.

One form of the invention is illustrated in the accompanying drawing which is a longitudinal 25 sectional view of a tracer bullet.

The bullet consists of the usual jacket 5 having a slug 6 in its front part and a cavity 7 in its rear part. A combustible loaded into the cavity or into a cup 8 placed therein, consists of a tracer composition 9 and an igniter mixture 10 which is adapted to be ignited from the propellant charge and to transmit ignition to the tracer composition.

The igniter mixture possesses the characteristic 30 of being invisible or non-tracing when the bullet is in flight and its quantity and rate of burning will determine the point in the trajectory at which ignition is transmitted to the tracer composition which when burning is clearly visible. As an example, in a .30 caliber bullet, 2.5 grains of the particular igniter mixture to be disclosed herein provides a delay corresponding to the first 250 yards of the trajectory.

An igniter mixture capable of functioning in 35 the manner outlined consists of a resinate of an alkaline earth metal such as calcium 5—20%, a

peroxide of an alkaline earth metal such as strontium 70—90%, and a metallic fuel such as magnesium 0—10%. The resinates and peroxides of other metals may be combined to impart the property of invisibility. The magnesium may be omitted, or other metals or fuels added to modify the properties. Oxidizers may also be added to the mixture in order to modify the burning characteristics.

A particular example of an igniter mixture 10 which is invisible when burning is as follows:

|                    | Percent |
|--------------------|---------|
| Calcium resinate   | 5       |
| Strontium peroxide | 90      |
| Magnesium          | 5 15    |

These ingredients are blended dry and loaded on top of the tracer composition in a suitable press. An alternative method of blending consists in first wetting the calcium resinate and strontium peroxide with carbon tetra-chloride. After mixing the whole thoroughly it is poured into shallow pans and dried at a gentle heat. The dried cake is then granulated to the desired fineness and the magnesium added. The igniter prepared in this manner is generally more stable than the igniter made by blending the dry ingredients.

We claim:

1. A delay non-tracing igniter mixture for tracer ammunition comprising calcium resinate 30 5%, strontium peroxide 90%, magnesium 5%.

2. A delay non-tracing igniter mixture for tracer ammunition comprising calcium resinate 35 5—20%, strontium peroxide 70—90%, and magnesium up to 10%.

3. A delay non-tracing igniter mixture for tracer ammunition comprising a resinate of an alkaline earth metal 5—20%, a peroxide of an alkaline earth metal 70—90%, and a metallic fuel up to 10%.

4. A delay non-tracing igniter mixture for tracer ammunition comprising calcium resinate 40 5—20%, strontium peroxide 80—95%.

THOMAS STEVENSON. 45  
ERNEST R. RECHEL.